

## UNITED STATES PATENT OFFICE

CHARLES A. BUERK, OF CHICAGO, ILLINOIS

## LIQUID COMBUSTIBLE

No Drawing.

Application filed May 4, 1936. Serial No. 103,758.

This invention relates to improvements in hydrocarbons, such as benzol, gasoline, naphtha, kerosene, crude oil, and in fact all of the so-called coal tar derivatives, also 5 oxygen-containing fuels, such as alcohol, both ethyl and methyl, and the like used for generating power by combustion, particularly in an internal combustion engine.

The invention consists in the addition or 10 admixture of a compound containing oxygen such as benzoyl peroxide, hydrogen peroxide, or naphthaline peroxide, or various persalts, or a combination or mixture thereof to the more commonly used forms, such as 15 gasoline, benzol, naphtha, kerosene, crude oil, and crude oil derivatives and also alcohol, both ethyl and methyl.

I have found that by adding a compound 20 containing oxygen with the above named well known products, and particularly by adding such compounds having an extra atom of oxygen, an improved explosive combustible is obtained which not only increases the power of a combustion engine but also 25 that a cleaner combustion is obtained which does not result in the formation of carbon on the interior of a combustion engine, and in fact if this improved material is used in a combustion engine in which there is carbon, 30 the carbon deposits will gradually decrease and will eventually disappear.

The ingredient which is preferable is benzoyl peroxide, which may be described as an oxygen carrying agent, which is a comparatively 35 inexpensive product that may be added in proportions from three-fourths ( $\frac{3}{4}$ ) of an ounce to one-half ( $\frac{1}{2}$ ) ounce for thirteen (13) gallons of commonly used explosive, either more or less, depending upon 40 the effect desired and the result with such an admixture is that the known hydrocarbon or other fuels is given an increased and quicker explosive effect, thereby resulting in greater power and having a carbon removing 45 effect as previously set forth.

Benzoyl peroxide has the formula:



50

It is to be understood that the essential component of the grouping is the radical  $-\text{O}-\text{O}-$  which is characteristic of peroxides. In benzoyl peroxide the radical



55

is a typical grouping which may occur in other peroxides having other radicals corresponding to the phenyl radical  $\text{C}_6\text{H}_5-$ . Although benzoyl peroxide has two similar phenyl radicals, this similarity is by no means necessary.

There is a particular advantage in using 65 compounds such as benzoyl peroxide. In benzoyl peroxide there are found only the elements carbon, hydrogen and oxygen. These are the three elements involved in the combustion of ordinary fuels. Furthermore, 70 these elements all form gaseous products of combustion which merely add to the products from the fuel in quantity rather than in kind. There is, therefore, no danger of introducing foreign or deleterious combustion 75 or reaction products into the engine.

It is a characteristic of the oxygen-containing substances of this invention that they release active oxygen. This release is effected in a variety of ways, among them 80 the application of heat. It is possibly this latter effect which releases the active oxygen contained in benzoyl peroxide when the latter enters the combustion chamber. It is well known that oxygen from such substances is distinguished from the oxygen of the air by its greater activity. When released in the presence of combustible material it is without doubt preferentially consumed in the preliminary stages of combus- 85 90

tion, and in a manner beneficial to the combustion. In addition to the oxygen released, other products are formed by the decomposition of the benzoyl peroxide which may also have beneficial effects.

It is found in practice that mixtures of this material produce no dangerous or detrimental effects; they may be used wherever the original unaltered fuel is used, the improved result being due, it is believed, to the added oxygen in the new mixture thus formed. The mixture of increased quantities of the additional oxidizing agent will produce an additional explosive effect, but too rich a mixture is objectionable from a commercial standpoint. Furthermore it is believed that other materials may be used as an oxidizing agent for well known combustibles without departing from the spirit and scope of my invention.

I claim:

1. The combination of a combustible fuel such as a hydrocarbon, gasoline, crude oil and liquid alcohols used for generating power by combustion with benzoyl peroxide in a comparatively small quantity to produce reaction products having a better combustible effect than the original combustible material when used alone.

2. The method of increasing the combustibility of a liquid hydrocarbon used for generating power by combustion which consists in adding thereto a small percentage of benzoyl peroxide which increases the oxygen in the mixture to such an extent that it has an increased intensity as an explosive mixture.

3. The combination with a liquid combustible, such as gasoline, crude oil and alcohol, of benzoyl peroxide in the proportion of from three-fourths ( $\frac{3}{4}$ ) to one and one-half ( $1\frac{1}{2}$ ) ounces of peroxide to three (3) gallons of the combustible.

4. The combination of a liquid hydrocarbon, and a small percentage of benzoyl peroxide intimately mixed therewith and producing an explosive effect.

5. The combination of a combustible fuel such as gasoline, crude oil and liquid alcohols used for generating power by combustion with an organic peroxide in a comparatively small quantity to produce reaction products having a better combustible effect than the original combustible material when used alone.

6. A combustible fuel containing a small quantity of a material selected from the group consisting of benzoyl peroxide, hydrogen peroxide, naphthalene peroxide, and per-

60 salts.

CHARLES A. BUERK.